

## UNITED STATES PATENT OFFICE.

WENDELL R. SWINT, OF LONDON, ENGLAND, ASSIGNOR TO E. I. DU PONT DE NEMOURS & COMPANY, OF WILMINGTON, DELAWARE, A CORPORATION OF DELAWARE.

## LOW-DENSITY DYNAMITE.

No Drawing.

Application filed August 23, 1924. Serial No. 733,780.

This invention relates to the manufacture of explosives having a liquid sensitizing agent, and in particular to the manufacture of ammonium nitrate explosives of the permissible type.

In the mining of coal, it is at times important to obtain the maximum possible proportion of lump product. For the production of this type of product, it has become recognized that for economy in operation, the strongest possible explosive must be used, having at the same time the lowest possible velocity, and a density such as to give the proper distribution of explosive in the bore hole. With these properties must of course be coupled permissibility for use in coal mines, and sufficient sensitiveness to detonation to insure propagation of explosion throughout a single charge.

In the development of this type of explosive, the disclosures of Woodbury (U. S. P. 1,113,275 and 1,124,679) brought about a great step forward. By his method, the velocity of detonation is lowered by increasing the size of the granules of the nitrate of ammonia, the reduction in velocity being in general proportional to the increase in the size of the granules. This method of control of velocity has had definite limitations in that the use of a too coarsely granulated nitrate of ammonia will tend to interfere with the strength of the explosive, and with the known absorbents it has been difficult to obtain any material reduction in density (with consequent reduction in velocity) beyond certain rather definite limits without interfering seriously with the sensitiveness of the dynamite.

Explosives of the type described above have previously been made of such a density that a  $1\frac{1}{4}'' \times 8''$  cartridge has weighed 160 to 180 grams (126 to 142 sticks per 50 lbs.), and have in general been made with ammonium nitrate of such fineness that the major portion of the grains pass a 10 mesh, and are held on a 60 mesh screen. Ammonium nitrate of this degree of subdivision may be referred to as a relatively coarse ammonium

nitrate. An example of such a composition follows:

|                  | Per cent |
|------------------|----------|
| Nitroglycerine   | 10       |
| Ammonium nitrate | 80       |
| Wood flour       | 5        |
| Cornmeal         | 5        |
|                  | 55       |

Many variations have of course been made in formulas of this type, as for example, the substitution of 3-20% sodium chloride for a corresponding proportion of the ammonium nitrate; the use of similar proportions of sodium nitrate in place of the ammonium nitrate; the substitution of other carbonaceous materials, such as starch, ivory nut meal, sawdust, wood pulp, for the wood flour and cornmeal; and the use of other explosive liquids as substitutes for all or part of the nitroglycerine; as well as various changes in the relative proportions of the several ingredients mentioned.

Using previously known materials and relatively coarse ammonium nitrate such as is described above, the lowest density it has been previously possible to obtain in explosives of this type corresponds to a weight of about 151 grains (150 sticks per 50 lbs.) in  $1\frac{1}{4}'' \times 8''$  cartridges, and this can be obtained only by the greatest care in the preparation and selection of materials.

The explosives manufactured from this type of coarse ammonium nitrate have in general had velocities below 2500 m/sec. In order to obtain lower densities than this, it has been necessary to use finer nitrate of ammonia, which in turn has caused an undesirable increase in velocity.

I have discovered that by the use of a new absorbent material to replace all or part of the carbonaceous materials previously used, I can obtain material reduction in the density of the resulting dynamite, without interfering to any serious extent with the explosive properties of the dynamite, and accompanied by an additional reduction in velocity over that normally obtained by the use of the coarse ammonium nitrate, due directly to the reduction in density obtained.

My new absorbent is obtained by the treatment of sugar cane in such a way as to recover the so-called bagasse pith. According to this treatment, the residue from the sugar cane, after the extraction of the sugar, said residue usually being in a crushed and macerated condition, is screened to remove the majority of the long fibers, leaving mainly the pith. Small percentages of the fibers do not interfere with securing the desired results, but the pith as used in my invention should preferably not contain over 25% fiber. Other methods of sugar manufacture in which the entire cane is first shredded and dried and then extracted with water to remove the sugar also may be utilized in obtaining bagasse pith of properties which are satisfactory for use in my invention.

The product thus obtained is a finely divided material having a distinct cellular structure, with very distinctive appearance when viewed under the microscope.

I may use this absorbent either as a partial or complete substituent for the carbonaceous materials previously used. For example, the following table shows one series of formulas illustrating the use of the new absorbent, though it is to be understood that the formulas here given constitute only a small proportion of the possible formulas in which the material can be used.

|                                    | Per cent. | Per cent. | Per cent. |
|------------------------------------|-----------|-----------|-----------|
| 35 Nitroglycerine                  | 10        | 10        | 10        |
| Relatively coarse ammonium nitrate | 75        | 75        | 75        |
| Sodium nitrate                     | 5         | 5         | 5         |
| Bagasse pith                       | 3         | 6         | 10        |
| Wood flour                         | 7         | 4         | —         |

The decrease in density obtained in the finished dynamite will of course vary with the extent to which the substitution of the new absorbent is carried. I have been able with such formulas to obtain average densities corresponding to as low a weight as 125 grams (181 sticks per case) for an 1 1/4" x 8" cartridge without seriously affecting the sensitiveness of the explosive. Considerably lower densities than this can be obtained by increasing the content of bagasse pith absorbent beyond the amount used in the above formulas. This change however must usually be accompanied by slight increases in nitroglycerine content in order that sensitiveness may be maintained, and this in turn will in certain cases necessitate the inclusion of additional safety ingredients,

for example NaCl or NH<sub>4</sub>Cl, replacing for example part of the ammonium nitrate.

The most important ranges in composition which are possible may be indicated as follows:—

|                                    | Per cent. | 65 |
|------------------------------------|-----------|----|
| Nitroglycerine                     | 7-15      |    |
| Relatively coarse ammonium nitrate | 40-85     |    |
| Sodium nitrate                     | 0-20      |    |
| Sodium chloride                    | 0-20      |    |
| Bagasse pith                       | 3-15      | 70 |

It is understood that there may be substituted other liquid explosive materials for part or all of the nitroglycerine; for example, tetrinitrodiglycerine or ethylene glycol dinitrate that there may be used any of the well recognized methods for depressing the flame temperature in order to obtain an explosive permissible for use in coal mines, and that there may be used bagasse pith either alone or in conjunction with other carbonaceous materials without departing from the invention.

I claim:

1. A dynamite comprising relatively coarse ammonium nitrate, bagasse pith and a liquid explosive ingredient, having a density such that an 1 1/4" x 8" cartridge will weigh less than 146 grams, and having a velocity less than 2500 m/sec.

2. A low velocity dynamite comprising 50 to 80 per cent of relatively coarse ammonium nitrate, bagasse pith and a liquid explosive ingredient, and having a density such that an 1 1/4" x 8" cartridge will weigh less than 146 grams.

3. A low velocity dynamite comprising 50 to 80% relatively coarse ammonium nitrate, bagasse pith and 7 to 15% of a liquid explosive ingredient, and having a density such that an 1 1/4" x 8" cartridge will weigh less than 146 grams.

4. A low velocity dynamite comprising relatively coarse ammonium nitrate, a liquid explosive ingredient and bagasse pith.

5. A low velocity dynamite comprising relatively coarse ammonium nitrate, nitroglycerine, and bagasse pith.

6. An ammonium nitrate dynamite of a velocity less than 2500 m/sec., the velocity being reduced by the incorporation of the ammonium nitrate in the form of coarse crystals and also by the presence of bagasse pith.

In testimony whereof I affix my signature.

WENDELL R. SWINT.